

May 3, 1927.

A. KÄMPF ET AL

1,627,037

METHOD OF LOOSENING PARALLEL FIBER BUNCHES BY THE WET PROCESS

Filed Oct. 16, 1925



*Inventor.  
Adolf Kampf and  
Karl Grunewalder*

*By: Marks & Clark  
Atty's*

## UNITED STATES PATENT OFFICE.

ADOLF KÄMPF AND KARL GRÜNEWÄLDER, OF PREMNITZ, WESTHAVELLAND, GERMANY.

## METHOD OF LOOSENING PARALLEL FIBER BUNCHES BY THE WET PROCESS.

Application filed October 16, 1925, Serial No. 62,906, and in Germany December 18, 1924.

In recent times the tendency has arisen to replace cotton by other spinning fibers. In particular two processes have been suggested for this purpose: In the first place 5 the cottonizing of certain fibrous waste materials, hemp shives and the like which have hitherto been more or less worthless and in the second place the manufacture of fibrous material capable of being spun on cotton 10 machines, which is obtained by chemical means, that is to say, in the manner of artificial silk. A special importance is in both these cases attached to the problem of loosening the individual fibers from one another as 15 completely as possible in order that the spinning may be carried out easily and without damaging the fibrous material.

In the cottonizing of natural fibrous waste materials use is made for the purpose of 20 loosening the individual fibers from one another of known devices by means of which the fiber bunches coming out from between rollers are worked up with sharp jets of water and are thus pulled to pieces. It is 25 also comparatively expensive in providing the apparatus and in working.

The invention consists in suspending the fiber bunches in a suitable liquid, hot soap suds for example, and this suspension is now 30 allowed to fall freely against impact surfaces. The kinetic energy of the splashing water is in this case also operative upon the parallel fiber bunches and the latter are loosened. This action can be enhanced in 35 a convenient manner by the fact that with a suitable height of fall of the suspension, the process is repeated as often as may be desired, the suspension being allowed to rush down from one impact surface to the next 40 in succession. The fibrous material is preferably added to the liquid in uniform quantities at the commencement of the downward flow. In this way the risk is obviated of certain quantities of fiber prematurely 45 floating free from one another and encircling the fiber bunches like a net, which leads to an irregular loosening. The fibrous material is finally taken out, centrifuged or squeezed and dried.

The process is characterized by the fact 50 that it is particularly well adapted for the treatment of artificial fibers.

In the accompanying drawing a piece of apparatus suitable for carrying out the process is diagrammatically illustrated by way 55 of example.

The fibrous material passes through a cutting device *a* on to a conveying band *b*, which brings the material to the upper mouth of a tower *d*. At *c* the liquid, for 60 example soap suds, enters and flows together with the fibrous material into the tower and on to the impact surfaces one after another. At *f* the fibrous material treated enters for 65 example a hydroextractor *g*.

Having now particularly described and ascertained the nature of our said invention and in what manner the same is to be performed, we declare that what we claim is:—

1. A method of loosening parallel fiber bunches by the wet process, comprising suspending said fiber bunches in a suitable liquid and letting the suspension fall freely against impact surfaces.

2. A method of loosening parallel fiber bunches by the wet process, comprising suspending said fiber bunches in a suitable liquid and letting the suspension fall freely and repeatedly against impact surfaces.

3. A method of loosening parallel fiber bunches by the wet process, comprising suspending said fiber bunches in soap suds and letting the suspension fall freely against impact surfaces.

4. A method of loosening parallel fiber bunches by the wet process, comprising suspending said fiber bunches in soap suds and letting the suspension fall freely and repeatedly against impact surfaces as and for 90 the purpose set forth.

In testimony whereof we have signed our names to this specification.

DR. ADOLF KÄMPF.  
KARL GRÜNEWÄLDER.